

# UNITED STATES PATENT OFFICE.

CHARLES PACK, OF BROOKLYN, NEW YORK, ASSIGNOR TO DOEHLER DIE CASTING COMPANY, OF BROOKLYN, NEW YORK, A CORPORATION OF NEW YORK.

## MOLD.

1,301,965.

Specification of Letters Patent. Patented Apr. 29, 1919.

No Drawing.

Application filed January 5, 1917. Serial No. 140,711.

To all whom it may concern:

Be it known that I, CHARLES PACK, a citizen of the United States, residing at the borough of Brooklyn, in the city of New York, county of Kings, and State of New York, have invented certain new and useful Improvements in Molds, of which the following is a specification.

My invention relates to molds and more particularly to a type of mold made of plastic material adapted to be used in the casting of fluid metals.

Molds of the character to which my invention relates are used in the production of intricate castings requiring little or no machining after being drawn from the mold and having sufficiently exact dimensions to permit them to be incorporated in the different mechanisms without requiring material machine work thereon. Castings made in such molds possess all of the surface characteristics of finished castings produced by what is known as the pressure die casting process as to accuracy of dimensions and finish.

Heretofore in the production of molds for making such castings, it has been the practice to employ a mixture composed of the ordinary commercial plaster of Paris and powdered asbestos either with or without a fibrous fusible binder for the purpose of securing greater tenacity in the body of the mold, or through the burning out of said fibrous material to form ducts to secure a more rapid venting of the mold during the pouring operation. In making the molds the mixture is formed in suitable frames about patterns which may be made of metal or of low fusing material such as wax. I have found in producing molds of this character, there is a tendency of the plastic to imprison air in and about the surface of the pattern, particularly where sharp angles or depressions are presented in the pattern, thus necessitating the agitation of the plastic mass about the pattern to free any such imprisoned air and secure exactitude in the mold cavity. By experiment, I have discovered that the composition consisting of asbestos and plaster of Paris is not suitable for the production of molds of this character because the mixture cannot be satisfactorily handled except when it has thickened or become partially set by reason of the tendency of water in excess of that required in form-

ing a combination with the solids of the plastic material, to stratify and come to the top of the mold.

Furthermore, I have found it necessary to use a composition which may be poured into the frame in a fluid or viscous condition to permit the agitation thereof about the pattern in a manner to prevent the formation of bubbles or blow-holes upon the surface of the cavity into which the metal is to be poured. With the asbestos and plaster of Paris composition, if the mass be sufficiently fluid to permit of its agitation as above referred to, the water will not only accumulate at the top of the mold being formed in the manner above referred to, but the plaster of Paris will be precipitated, forming a stratum at the bottom of the mold, the asbestos constituent forming a stratum intermediate the plaster of Paris and the water which stratum is too weak to withstand the stresses incidental to the casting operation and which rapidly cracks in a manner to form fins upon the casting which fins make the casting difficult to remove, and necessitate complicated machine re-finishing of the castings. Furthermore, the stratum of plaster at the bottom of the mold is very much less porous than the stratum of asbestos and has a tendency to warp during the drying out of the mold prior to the casting operation. This condition also results in a mold, different portions of which not only have different degrees of porosity but have variable conductivity. A mold made from a composition of plaster of Paris and asbestos, while being suitable for many purposes, is not suitable for use in the production of commercial metal castings of mechanical parts by reason of the lack of homogeneity of the mold in its entirety and the resultant conditions in the mold made therefrom above referred to.

With these conditions in mind, the object of my invention is to provide a mold of plastic material, the nature of the ingredients of which will be such as to have an affinity for each other and have absorptive properties which will avoid the stratification of excess water and of the solid ingredients entering into the composition.

A mold made in accordance with my invention, when the composition sets, will have substantial homogeneity throughout the entire body thereof and the patterns

may be drawn therefrom in a manner to leave smooth surfaces and sharp edges owing to the tenacity of the material of the mold which will be sufficiently great to prevent the breaking or chipping of the material of the mold as a result of the force applied in removing the pattern. All parts of the mold will be sufficiently porous to admit a free venting during the casting operation and the uniform porosity of all parts of the mold facilitates the elimination of the moisture in the mold by heat drying without likelihood of the warping of the mold due to the necessity for a prolonged subjection of the mold to heat, after any portion thereof has been thoroughly dried.

In the production of a mold made in accordance with my invention, the ingredients I employ are such as to permit the pouring of the plaster, while in a fluid or viscous state, about the pattern or patterns and within a frame, and the subsequent agitation of the plastic material about the pattern or patterns in a manner to expel the air and thus insure the smooth surfaces in the finished mold.

Furthermore, the composition of the mold makes possible the separation of enough of the moisture, either free or in combination with the solids contained in the mold by a uniform application of heat without likelihood of prematurely drying portions thereof with a resultant warping or distortion of the portions of the molds which are the first to lose their moisture.

The invention consists primarily in a mold formed of plaster of Paris and a granular, porous, non-fibrous and absorptive material having an affinity for plaster of Paris; and in the novel steps and practices in making said mold all as hereinafter set forth and described and more particularly pointed out in the claims hereto appended.

In the practice of my invention, I form a mold consisting of pulverulent silicious sinter, also called kieselguhr, and cellite, mixed with ordinary commercial plaster of Paris and a suitable fluid such as ordinary water in such proportions as to secure the desired condition of the mixture. In practice, I have found the most satisfactory results are secured by using equal quantities by bulk of kieselguhr or cellite and plaster of Paris, using enough water to make the composition sufficiently fluid to readily flow. I do not desire, however, to limit myself to the exact proportions stated, as the proportions may be varied. I have found that the kieselguhr or cellite has a strong affinity for the plaster of Paris, and that the solids entering into the composition absorb and retain moisture far in excess of that which will enter into combination therewith.

In making the molds, I mix the plaster of

Paris and kieselguhr or cellite while dry and add thereto the desired volume of water, thoroughly mixing the composition. The mixture is then poured into a frame having placed therein one, or a number of patterns, and by reason of its fluidity, the composition flows freely about each of the patterns and throughout the frame. After being so poured, it will remain fluid for a sufficient time to permit the molder to agitate the plastic about each pattern in a manner to free any imprisoned air and cause the fluid composition to closely hug the pattern. The composition is then allowed to set and thereafter the pattern is drawn therefrom. I have found that in setting, a composition, such as I have described, does not stratify but solidifies into a substantially homogeneous mass of substantially uniform density or porosity, and that the material is sufficiently tenacious to permit the drawing of the pattern while the molding material is still wet without providing any substantial draft in the patterns to avoid a break down of the walls in or about the mold cavity. This tenacity in the mold is highly desirable where split molds are used, although a matter of secondary importance where fusible patterns are employed. The other characteristics of the mold are of equal importance, however, irrespective of the type of mold made.

After the patterns have been drawn, the mold is subjected to the action of heat for a sufficient time and at sufficiently high temperature to not only remove the free moisture, or the moisture in suspension, in the mold but also that moisture which has combined with the solid ingredients of the mold, thus avoiding likelihood of injury to the mold when the molten metal is poured thereinto. The casting or castings are drawn from the mold by breaking the mold from about same after they have solidified.

The absorptive properties of the mold, result in uniformity in the drying action through all parts of the mold, thus avoiding likelihood of the distortion or working of small parts of the mold about the cavity therein.

While the outside of the mold has a tendency to dry first, nevertheless, the properties above referred to will gradually bring moisture to the surface of the mold and this drying of the outside will not have a tendency to injure the molds in any way.

The non-conductive properties of a mold made in accordance with my invention prevent a too rapid chilling of the lighter portions of the castings while the uniform porosity affords ample venting of the mold without the necessity for providing special vent openings.

A completed mold made in accordance with my invention is substantially devoid of

all moisture thus presenting an article consisting solely of the solid constituents entering into the composition of the mixture from which it is made.

- 5 Furthermore, while the mold possesses the desired characteristics of low conductivity and porosity desirable in molds of this character, the chief advantage in the use of the composition herein described is the ability 45  
 10 to work the composition in making the molds in a manner to secure exactitude in the formation and dimensions of the mold cavity by reason of the possibility of using the composition while in a fluid or viscous condition  
 15 without likelihood of stratification of the different ingredients when the mold sets. Furthermore, kieselguhr or cellite or an equivalent silicious sinter, possesses superior qualities in that it is granular, porous, non-fibrous, absorptive and has an affinity for 50  
 20 the plaster of Paris. In addition to these characteristics it has a low specific gravity and is sufficiently bulky to be more economical in use than asbestos or similar material.  
 25 It is not my intention to limit the invention to the exact proportions herein referred to nor to the exact manner of mixing the kieselguhr and the plaster of Paris, it being apparent that such proportions and the manner 55  
 30 of mixing same may be varied without departing from the spirit and scope of the invention.

Having described the invention what I claim as new and desire to have protected by 60  
 35 Letters Patent is:—

1. A mold adapted for the production of intricate finished metal castings formed of plaster of Paris and a granular, porous, non-fibrous, absorptive material having an affinity 65  
 40 for plaster of Paris, the material of said mold being devoid of free moisture and

moisture normally combined with the solids thereof, the composition of the mold being a substantially homogeneous mass of substantially uniform density.

2. A mold adapted for the production of intricate finished metal castings formed of plaster of Paris and cellite, in a substantially homogeneous mass of substantially uniform density. 45  
 50

3. A mold adapted for the production of intricate finished metal castings formed of plaster of Paris and a silicious sinter, the material of said mold being devoid of free moisture and moisture normally combined 55  
 55 with the solids thereof, in a substantially homogeneous mass of substantially uniform density.

4. A mold adapted for the production of intricate finished metal castings formed of plaster of Paris and a silicious sinter in substantially equal quantities of bulk, the material of said mold being devoid of free moisture and moisture normally combined with the solids thereof in a substantially homogeneous mass of substantially uniform density. 60  
 65

5. A mold adapted for the production of intricate finished metal castings, formed of plaster of Paris and cellite in a substantially 70  
 75 homogeneous mass, the material of said mold being substantially free from free moisture and moisture normally combined with the solids thereof.

In witness whereof I hereunto affix my signature in the presence of two subscribing witnesses, this 28th day of December, 1916.

CHARLES PACK.

Witnesses:

CHARLIE FEIT,  
 Wm. G. GUTMUELLER.